

## UNITED STATES PATENT OFFICE

2,467,233

TREATMENT OF WOOL AND PRODUCTS  
THEREFOR

John B. Rust, East Hanover, N. J., assignor to  
Montclair Research Corporation, a corporation  
of New Jersey

No Drawing. Application September 3, 1946,  
Serial No. 694,675

5 Claims. (Cl. 260—29.4)

1

The present invention relates to the treatment and shrinkproofing of wool and wool containing fibers, to the methods for obtaining such treated and shrinkproofed fibers, to the materials and products resulting from such processes and treatments, and to the baths and materials utilized to accomplish these results as well as methods of preparing such baths and materials.

Urea formaldehyde type resins under which there may be included such synthetic resins as mono- or di-methylol urea or mixtures thereof, urea formaldehyde or alkylated urea formaldehyde condensation products, melamine formaldehyde resins and their alkylated modifications, such as for instance, the types known to the trade as "Lanaset" or "Resloom," have been utilized in the treatment of textiles and fabrics for the purpose of crease-proofing or improving draping qualities of fabrics and textiles. Such agents are very inferior as shrinkproofing agents for wool and have little effect per se on such shrinkproofing unless cured at high temperature, but such control is usually accompanied by a degree of harshening of the fabric.

In prior applications more particularly identified below, the art has been taught that butadiene-1,3 and some of its copolymers produce superior shrinkproofing effects on wool and related materials. In some cases there is a slight "sticky" or "greasy" hand imparted to the goods which may be objectionable depending on the particular utilities for which the materials are employed.

Among the objects of the present invention is the treatment of wool and wool containing materials to render the treated material substantially resistant to fulling, felting, or shrinking without damage to the fabric or fibers, and at the same time preserving the desirable hand of such materials as well as retaining favorable wearing qualities.

Other objects of the present invention include shrinkproofed wool and wool containing fabrics.

Other objects include the treatment of wool and wool containing materials to improve their draping qualities.

Further objects include the treating baths and materials required for the purposes set forth above, as well as methods for producing such materials.

Still further objects and advantages of the present invention will appear from the more detailed description set forth below, it being understood that this more detailed description is given by way of illustration and explanation only, and not by way of limitation, since various changes therein may be made by those skilled in the art without departing from the scope and spirit of the present invention.

In accordance with the present invention, the wool or wool containing fibers, which may be of

2

various types, is treated with an emulsion more particularly an aqueous emulsion or dispersion, of a synthetic butadiene-1,3 polymer or copolymer in combination with aqueous solutions or dispersions of synthetic resins, such as for instance, mono- or di-methylol urea or mixtures thereof, urea formaldehyde or alkylated urea formaldehyde condensation products, melamine formaldehyde resins or their alkylated modifications, such as for instance, the types known to the trade as "Lanaset" or "Resloom."

It has been found that the combination of these two classes of materials not only improves the hand of the goods, but also quite unpredictably that certain unexpected improvements in the shrinkproofing characteristics accrue and there are also additional important qualities obtained such as improved draping, etc.

The wool treated may be of any desired type, such as raw wool, yarn, knitted or felted fabrics, woven or mixed goods, or combination fabrics including wool in various ways.

The wool may be treated with the treating emulsions, dispersions or solutions in any desired way, as by immersing the wool in the treating bath, or padding the treating bath on the wool, or by exhaustion of the polymer onto the wool, etc., various methods being more particularly illustrated below. And the sequence of the application of the resin and polymer components may be altered depending on the results desired. Thus if a finish is desired which has a certain "tack" to it, it may be desirable to treat the goods first with the resin and then with the polymer. On the other hand, if a stiffer finish is desired, the procedure may be reversed, first treating the goods with the polymer and then with the resin. Or combinations may be employed in which the treating bath includes both the resin and the polymer. An exceedingly simple and rapid method consists in a padding operation whereby both the resin and the elastomeric components are applied simultaneously from the same bath, followed by the required amount of curing. Where the treatment is carried out by successive applications of the treating baths containing resin and polymer or polymer and resin, there may be intermediate treatments, as for example, where after treatment with resin with or without curing, the treated material is then subjected to an intermediate step of acidification or treatment with an acid solution before the application of the polymer bath.

Any of the urea formaldehyde type resins under which all of the modifications set forth above are included, may be utilized so that at least one of the urea formaldehyde and melamine formaldehyde resins is employed and in the final product is in cured condition. Such urea formaldehyde type resins are generally applied in the

form of aqueous solutions and the application may be made simply by immersing the goods in this solution and removing the excess liquor by squeezing or by extraction. Or, in the case of fabrics, these may be padded and the excess liquor removed by passing the impregnated fabric through squeeze rolls. The strength of the pad liquor is dependent upon and determined by the amount of resin which it is desired to deposit on the fabric, as well as by the amount of liquid pick-up of which the fabric is capable.

The amount of resin applied to the goods is determined by the desired effect but will be generally limited between 1 and 25% on the weight of the fabric treated. A suitable curing catalyst such as ammonium phosphate, ammonium sulfate, etc., is desirably added to the solution containing the resin in order to facilitate curing. The fabric may then be dried at any suitable drying temperature ranging between room temperature and 100° C. and then cured. Alternatively, the fabric may be exposed to the curing temperature at once. The curing temperature, as well as the time required to complete the cure differs for various resins, and is conditioned also by the presence, quantity and kind of catalyst used. The curing temperature may vary between room temperature and 150° C. and the time required may range from 5 minutes to several days. It is important to note that materials may be employed which cure at room temperatures in reasonable periods of time so that elevated temperatures and long periods of treatment are not essential but may be employed.

The butadiene-1.3 polymer or copolymer may be applied to the fabric in various ways. Thus the aqueous polymeric dispersion may be diluted to such an extent that the finished fabric will contain from 1 to 25% of the polymer. The goods are simply padded through this liquor or the material is treated by immersion. The excess liquor is removed either by squeezing or by centrifugal extraction. The bath may be conditioned with ammonia, wetting agents including long chain alcohol sulfates such as sodium lauryl sulfate, soaps and the like. In some cases it may be both possible and advisable to adjust the pH of the pad liquor below 7 in order to cause partial agglomeration, using acetic acid, sulfuric acid, phosphoric acid and the like, for this purpose. After padding, it is only necessary to dry the fabric at any desired temperature in order to set the polymer, that is, to form a stable bond between it and the fiber. On the other hand, the dispersion may be discharged on the fiber from a suitable bath, such a bath consisting essentially of an aqueous dilution of the polymeric dispersion to which has been added suitable conditioning electrolytes and the pH of which has been adjusted below 7, such a bath being stable at room temperatures unless in contact with receptive fibers. As such conditioning electrolytes, water-soluble salts may be used. The treatment is carried out by immersing the fibers or fabrics in this bath until exhaustion is complete. The temperature of the bath may be at room temperature but more desirably is kept between 40° C. and boiling. The rate of exhaustion is regulated by the temperature as well as by the concentration of the electrolytes. After the bath has cleared up substantially or completely, the goods may be removed, rinsed and dried.

In application Serial No. 537,537, filed May 26, 1944, now Patent 2,447,538, of which the present application is a continuation-in-part, and in

which there is more particularly claimed the shrinkproofing of wool by the utilization of aqueous baths containing a synthetic butadiene polymer, an emulsifying agent and a conditioning electrolyte, the bath desirably having a pH below 7, there is disclosed the utilization of butadiene polymers and polymers of its homologues to give superior non-felting effects. It has been found that the use of straight butadiene polymers or butadiene homologue polymers, that is, those in which the butadiene or the butadiene homologue is the sole polymer, gives superior non-felting and wool shrinkproofing than do the butadiene copolymers. The polymeric butadiene derivatives are those of butadiene-1.3 and its lower homologues, such as butadiene-1.3, isoprene, dimethyl butadiene, ethyl butadiene, ethoxy and methoxy butadiene, cyanobutadiene, particularly such derivatives of butadiene-1.3. As there set forth, copolymers of butadiene or butadiene homologues as set forth above may be utilized as long as the added component in producing the copolymer is not present in an amount which interferes with the desired shrinkproofing effect. Such added copolymerizing materials include the methacrylates and acrylates, such as methyl methacrylate and vinyl compounds generally including vinyl acetate, methyl methacrylate, ethyl acrylate, styrene, acrylonitrile, vinyl pyridine, methacrylonitrile, isopropenyl methyl ketone, vinyl phenyl ketone, vinyl methyl ketone, and the like.

As further set forth in said application, the electrolyte content of the bath emulsion or dispersion may vary over substantial limits but sufficient electrolyte should be present to condition the bath so that the bath although stable in the absence of wool fibers, will deposit the polymer in the presence of the conditioning electrolyte. Generally the electrolyte content for this purpose will vary between about 25% to about 5000% based on the weight of polymeric butadiene derivative present. As such electrolyte, water-soluble salts may be used, desirably such salts which do not precipitate the polymer. The following are exemplary: sodium sulfate, sodium chloride, sodium bromide, sodium iodide, sodium phosphate, sodium sulfamate, sodium sulfite, sodium bisulfate, sodium bisulfite, sodium nitrate, sodium acetate, and the like, and similar salts of the other alkali metal group including those of potassium, lithium, caesium, and so on. Salts like zinc chloride may also be used where the coagulation does not appear to be too serious since it occurs in small particulate form, and the particles may be redispersed by stirring. Neutral salts, specifically salts of strong bases and strong acids, particularly inorganic salts, are preferred. They may be generally characterized as substantially neutral highly ionizing salts.

The operation of applying the polymer is desirably carried out at temperatures ranging from 40° C. to the boiling point of the bath. The process may be applied before or after fulling, weaving, scouring and the like operations. In some cases it may be applied in the dye bath. Mixed goods including wool-cotton, wool-rayon, etc., can be treated by the methods without any deleterious effect. The wool may be subjected to a pretreatment of any desired type, as for example, chlorination or bromination before being treated in accordance with the present invention.

As further set forth in said prior application, the emulsions containing the butadiene polymer

may include any anionic emulsifying agent which is stable at a pH below 7. Such emulsifying agents are exemplified by sodium lauryl sulfonate, sodium alkyl naphthalene sulfonates, long chain alkyl sodium sulfonates, sodium dioctyl sulfosuccinate, etc. There may also be used neutral non-cationic emulsifying agents such as mannitol monolaurate, the reaction product of protein degradation products with acid chlorides, ethylene oxide reaction products with fatty acid, fatty alcohols, and the like.

As further set forth in said application, the emulsions of the polymer used are desirably but not necessarily, those which have been carried to a 100% polymerization. When 100% polymerization is obtained, considerable cross-linking has occurred in the polymer with consequent insolubility in organic solvents. Thus a type of pre-vulcanization of the polymer has been obtained. It is also possible to vulcanize the polymers with vulcanizing accelerators such as thiuram disulfite, etc., vulcanizing agents such as sulfur, di-nitrobenzene, alkyl phenol sulfide, etc., either previous or subsequent to deposition or dyeing, into the wool fibers.

As pointed out immediately above, the polymer employed is in a condition in which if deposited from the emulsion or dispersion, the polymer is in a substantially non-tacky condition and gives a non-tacky deposit. It is substantially insoluble in organic solvents but may be swollen to some extent with such solvents. It is in a condition in which it is totally unsuitable as synthetic rubber or rubber-like material since if coagulated by any suitable means it gives crumbly materials which cannot be milled on rubber milling equipment and which are entirely composed of cross-linked polymers. Any of the polybutadiene-1.3 compositions as set forth in said prior application may be utilized as the component for this phase of the treatment of the present invention.

While as pointed out in said prior application, straight butadiene polymers and butadiene homologue polymers are preferred, in order to obtain special effects certain additions and modification may be made to a limited extent. These additions may consist of other polymers in the form of emulsions, dispersions, factices, etc., and may include chloroprene polymer, polyvinyl compounds, polyacrylates such as polyethylacrylate, polyalkylmethacrylates, polystyrene and its derivatives such as alpha beta dimethylstyrene, dichlorostyrene, acrylonitrile, methacrylonitrile, etc. While it is understood that the addition of these auxiliary substances usually is limited to the extent where no substantial interference with the shrinkproofing characteristics is experienced, in special applications it may be desirable to exceed those proportions.

Thus in application Serial No. 563,791, filed November 16, 1944, entitled Treatment of wool, now Patent 2,447,539, there is more particularly claimed the treatment of wool by utilization of copolymers of a butadiene-1.3 and a methacrylate ester such as methyl methacrylate, ethyl methacrylate, and butyl methacrylate, in aqueous emulsions of the character set forth above, the amount of methacrylate polymer being about 5 to 20% of the interpolymer, of the ethyl methacrylate being about 5 to 50% of the interpolymer, and of the butyl methacrylate being from about 5% to 40% of the interpolymer. Any of such materials may be utilized as the polymer component of the present invention.

In application Serial No. 586,293, filed April 3,

1945, entitled Wool treating products and methods, now Patent 2,447,876, there is more particularly claimed the utilization of butadiene polymers in aqueous dispersions where soap is the essential or only emulsifying agent present, the pH of the bath being at least 7 and the soap being an alkali salt of a long chain carboxylic acid. Such baths and wool treated in accordance therewith may be utilized as the polymer treatment phase of the present invention.

In application Serial No. 586,637, filed April 4, 1945, for Pre-shrunk and shrink-proofed wool, there is more particularly described and claimed the treatment of wool to obtain shrinkproofing by the utilization of butadiene-1.3 emulsions and related materials as set forth above in which operations the wool is subjected to a treatment to relax any stretched wool fibers to produce a pre-shrunk wool and such pre-shrinking operations and polymer depositions for shrink-proofing may be utilized in any order of steps successively or simultaneously. Those operations in connection with the utilization of polymer for shrink-proofing and also pre-shrinking operations may also be employed in accordance with the present invention.

In application Serial No. 594,585, filed May 18, 1945, entitled Interpolymer treatment of wool, now Patent 2,447,540, there is more particularly claimed the treatment of wool utilizing a copolymer of butadiene and an acrylate ester, more specifically a methyl acrylate not exceeding 40% of the copolymer, an ethyl acrylate in an amount not exceeding about 50% of the interpolymer, and a butyl acrylate not exceeding about 60% of the interpolymer in the production of shrink-proofing treatments utilizing baths of the character set forth above. Any such compositions and baths and treatments may be employed in this phase of the invention of the present case.

In application Serial No. 613,200, filed August 28, 1945, entitled Elastomer production and utilization, now Patent 2,447,877, there is particularly claimed the production of shrinkproofed wool by the utilization of copolymers of butadiene-1.3 and a 2-methyl butadiene-1.3, specifically isoprene and 2,3 dimethyl butadiene-1.3, the copolymer being in the cross-linked condition as set forth above in which it is unsuitable for utilization for rubber but in its crumbly condition as utilizable in accordance with the shrinkproofing operations is particularly important for the treatment of wool. Such materials are described and claimed as employed in treating baths of the character set forth above. Any of such materials may be employed in accordance with the present invention for that phase of the treatment which includes the use of the polymer. Desirably as set forth in that prior case, the copolymer of butadiene-1.3 with isoprene is in the ratio of from 9:1 to 1:4 parts by weight, while that of the copolymer of butadiene with 2,3 dimethyl butadiene 1.3 is in the ratio desirably of 9:1 to 3:7 parts by weight. Such materials may be employed in the present invention.

In application Serial No. 613,201, filed August 28, 1945, entitled Butadiene copolymers and their utilization, now Patent 2,447,878, there is particularly described and claimed the treatment of wool for shrinkproofing by the utilization of copolymers of butadiene-1.3 and a benzene containing an unsaturated side chain of two carbon atoms such as styrene and its derivatives, namely, alpha, gamma-dimethyl styrene and dichloro-alpha, gamma-dimethyl styrene and dichloro-styrene as well as phenylacetylene, where the

7 copolymers are more particularly of the cross-linked character and if deposited per se from the emulsions would be crumbly materials unsuitable for rubber purposes. As set forth in such case, baths employing such materials of the character as set forth above may be utilized particularly where in the styrene copolymer, the amount of styrene does not exceed about 60% by weight of the copolymer, with the alpha, gamma-dimethyl styrene it does not exceed about 40% of the copolymer, whereas the dichlorostyrene does not exceed about 40% of the weight of the copolymer, but for phenylacetylene preferably not more than 20% by weight of the copolymer is present. Any of those materials may be utilized as the polymer phase of the present invention.

In application Serial No. 615,097, filed September 7, 1945, entitled Shrinkproofing wool and materials therefor, there is more particularly described and claimed the shrinkproofing of wool by the utilization of cross-linked copolymers of a butadiene-1.3 and an unsaturated ketone containing not more than 12 carbon atoms, having the formula  $\text{CH}_2=\text{CR}_2-\text{CO.R}_3$ , where  $\text{R}_2$  is selected from the group consisting of hydrogen, alkyl and aryl groups, and  $\text{R}_3$  is selected from the group consisting of alkyl and aryl groups, including more particularly copolymers of butadiene-1.3 with isopropenyl methyl ketone, methylene n-amyl methyl ketone, methylene isobutyl methyl ketone, etc., and where more particularly for shrinkproofing purposes in such copolymers the amount of isopropenyl methyl ketone does not exceed about 30% by weight of the copolymer, where methylene n-amyl methyl ketone is the copolymerizing material it does not exceed about 40% by weight of the copolymer, and when methylene isobutyl methyl ketone is the copolymerizing material, it does not exceed about 20% of the copolymer. Such materials may be utilized in emulsions, dispersions and baths as more particularly set forth above. Any such materials may be utilized as the polymer phase of the present invention.

In application Serial No. 615,098, filed September 7, 1945, entitled Woolshrinkage copolymers, there is more particularly described and claimed the utilization of cross-linked copolymers of a butadiene-1.3 and an acrylonitrile, such as acrylonitrile itself, methacrylonitrile, etc., more particularly where the weight of the acrylonitrile material either acrylonitrile per se or methacrylonitrile does not exceed about 40% by weight of the copolymer, such copolymers particularly being utilized in the cross-linked condition and employed in baths, aqueous emulsions and dispersions as set forth above. Any such materials may be utilized in the present invention for the polymer phase thereof.

In application Serial No. 631,483, filed November 28, 1945, entitled Elastomeric copolymers and their utilization, there is more particularly described and claimed the treatment of wool for shrinkproofing where there is utilized a copolymer of a butadiene-1.3 and a vinyl ester which polymerizes to a hard resinous material, more particularly such esters as vinyl acetate and vinyl chloride, desirably the vinyl acetate when employed not exceeding about 40% by weight of the copolymer, and the vinyl chloride also not exceeding about 40% by weight of the copolymer when it is employed. Such materials may be utilized in the shrinkproofing of wool by employment in aqueous baths, dispersions and emulsions as set forth above. Any such materials may be

utilized as the polymer phase of the present invention.

In application Serial No. 657,335, filed March 26, 1946, entitled Wool treatment and product, there is more particularly described and claimed the shrinkproofing of wool utilizing a synthetic chloroprene polymer, either alone or with limited amounts of other materials such as not exceeding about 50% of ethyl acrylate polymer based on the total weight of polymers present, or a vegetable oil factice not exceeding about 40% by weight of the polymer together with factice, or with methyl methacrylate polymer not exceeding about 40% of the total weight of polymers when this is used, or where the chloroprene polymer is utilized with a synthetic butadiene-1.3 polymer, or with a natural rubber latex, the latter, however, not exceeding about 75% of the total weight of polymer together with the latex present. Any 10 of these materials may be employed in the shrinkproofing of wool in the form of baths dispersions and emulsions as set forth above. The chloroprene polymer may also be utilized in the form of copolymers such as with an acrylonitrile 15 where the latter does not exceed about 40% of the total weight of the polymers present or with an ethyl acrylate copolymer, where the latter does not exceed about 50% of the total weight of the polymers present, or of a methacrylate polymer 20 not exceeding about 40% of the total weight of polymers present and again any of these materials employed in dispersions, emulsions or aqueous baths as set forth above. Any of these combinations may be utilized in accordance with the present invention as the polymer phase thereof.

In application Serial No. 603,406, filed July 5, 1945, entitled Textile and fiber treatment, compositions and methods, now Patent 2,447,772, 40 there is more particularly described and claimed the utilization of butadiene-1.3 polymers and combinations thereof with other materials as in aqueous baths, dispersions and emulsions for the shrinkproofing of wool where the butadiene component, that is, the synthetic butadiene polymer is employed in the form of a prevulcanized or preoxidized material, where the treatment has been carried to a point so that the polymer is present in a condition in which it will not give a 45 tacky deposit on fibers treated therewith. It is in substantially insoluble condition although it will swell with organic solvents as set forth above. Such prevulcanized or oxygen treated polymer emulsions, baths and dispersions may be employed in accordance with the present invention. Furthermore as set forth in that case and in other companion cases, antioxidants may be present not only to control any further oxidation or vulcanization which takes place and to 50 check the latter, but also because it has been found that antioxidants exert a very favorable effect of unexpected character on the shrinkproofing obtained. Thus antioxidants of the usual type may be employed in the dispersions or 55 emulsions in order to obtain the effects set forth above and any such materials may be utilized in accordance with the present invention as the polymer phase thereof.

Accordingly, in accordance with the present invention, wool of substantially normal hand is obtained but which has been shrinkproofed with a synthetic butadiene-1.3 polymer which may be of any of the characters set forth above, either by itself or copolymers of the character described above, utilized, however, in combination

with a cured urea-formaldehyde type resin. The amounts of polymer plus resin present in the treated material may vary from about 1 to 50% on the weight of the wool. Varying ratios of polymer to resin may be used, but in order to secure satisfactory shrinkage control, between 2 and 15% of polymer, based on the weight of the wool, should be utilized. A preferred ratio with urea formaldehyde resins varying from about 4:1 of urea formaldehyde type resin to polybutadiene to 1:1.2 of such resin to polybutadiene. Or preferred ratios with melamine type materials may run from about 3.1:1 of the melamine type resin to polybutadiene to 1:1.2 of the melamine or alkylated melamine type material. In all such cases where shrinkproofing is obtained, the amount of the polymer present should be generally at least 1% on the weight of the wool and the amount of any other materials present should not interfere with the shrinkproofing sought while other desired characteristics may be enhanced as pointed out above by the presence of such added materials.

The following examples illustrate the invention, the parts being by weight unless otherwise set forth.

*Example 1.*—A condensation product of urea-formaldehyde as well as butadiene polymer emulsion was applied to swatches of wool flannel, measuring 10" x 10" in size. The samples were immersed in the resin solution first and the excess pad liquor was removed by passing the fabric through squeeze rollers. The weight of the wool samples was noted before and after padding and from the weight increase the amount of resin applied to the fabric was calculated. The samples were dried at 60° C. and cured at this temperature for 12 hours. After curing the polybutadiene dispersion was applied in the same manner and the amount of polymer on the fabric was calculated as outlined above.

The solution of the urea-formaldehyde condensation product was prepared by dissolving equimolecular quantities of dimethylolurea and urea in sufficient water to form a solution containing 10% solids. To this was added 5% of ammonium sulfate based on the weight of the solids.

The aqueous polybutadiene dispersion was prepared as follows: butadiene was passed over calcium chloride and condensed in a pressure reactor cooled to below -5° C. 50 parts of butadiene were then weighed out in the reactor. While the reactor was kept in the freezing mixture, the following solution was added. 6 parts of soap (Ivory Flakes) was dissolved in 125 parts of water and the pH of the water-soap solution was adjusted to 10 by the addition of a small amount of 5% sodium hydroxide solution. The following catalysts and regulators were then added to the soap solution, 0.1 part of dodecyl mercaptan, 0.01 part of potassium ferricyanide, 0.2 parts of potassium persulfate. The reactor was then closed, allowed to come to room temperature and put in an agitator with a constant temperature bath at 45° C.

After 16 hours, the reaction was substantially complete as indicated by a very slight pressure within the reactor. The emulsion was then subjected to a vacuum of approximately 15 pounds per square inch to draw off the small amount of monomer gases that may be present. The polymer emulsion was then given an oxidation treatment as follows: added 1% of the sodium salt of sulfonated oleyl alcohol and 2½ of a 30% hydrogen

peroxide solution, then heated for one hour, the temperature rising gradually to 200° F. Since polymerization was almost complete, it was assumed that this dispersion contained 25% of polybutadiene.

This emulsion was diluted with water so that it contained 6% polybutadiene.

Four lengths of 8" each were marked on each sample, two in the direction of the warp and two in the direction of the fill. From these measurements the area in square inches was calculated. The wool samples were then washed for three hours in a mechanical washing machine, after which laundering they were rinsed, dried and remeasured.

The amount of resin and polybutadiene deposited on the fabric as well as the area shrinkage are shown below.

| Sample No.  | Percent Urea-formaldehyde Resin on Fabric | Percent Polybutadiene on Fabric | Percent Area Shrinkage |
|-------------|-------------------------------------------|---------------------------------|------------------------|
| 1           | 10                                        | 6                               | 29.6                   |
| 2           | 10                                        | 6                               | 4.2                    |
| 3           | 5                                         | 6                               | 13.0                   |
| 4           | 5                                         | 6                               | 1.0                    |
| 5           |                                           | 6                               | 3.5                    |
| 6 Untreated |                                           |                                 | 24.9                   |

The finished swatches had a dry, normal hand and the pieces which contained the urea-formaldehyde resin exhibited superior draping qualities.

*Example 2.*—A solution was made from equimolecular quantities of dimethylolurea and urea. The solution was diluted to a point where it contained 10% solids, to which was added 5% of ammonium sulfate, based on the weight of the solids. Four swatches of flannel were measured accurately and the area was calculated, after which they were thoroughly wet out with the urea-formaldehyde solution. The amount of liquid pick-up was determined by weighing the wool samples before wetting and after the excess pad liquor had been removed by passing the swatches through squeeze rollers. Of the samples, two were cured for 10 minutes at 125° C. and two were cured for 12 hours at 60° C.

One piece each, cured at a low and at a high temperature, as well as an untreated piece of flannel were then immersed in a polybutadiene dispersion, and after complete wetting out had taken place, the excess was removed by passing the goods through squeeze rollers, thereby removing the excess pad liquor. The polybutadiene solution was similar to the one used in the previous example, and the amount of solids deposited on the fabric was calculated as outlined above.

After drying, the samples were given a three-hour laundering. The amount of shrinkage, as well as a resume of the treatment which was given to the fabric may be found in the table below.

| Sample No.  | Per Cent Urea-formaldehyde Resin on Fabric | Cure            | Per Cent Polybutadiene on Fabric | Per Cent Area Shrinkage |
|-------------|--------------------------------------------|-----------------|----------------------------------|-------------------------|
| 1           | 17                                         | 12 hrs. 60° C.  | 6                                | 4.2                     |
| 2           | 17                                         | 10 min. 125° C. | 6                                | 4.6                     |
| 3           | 17                                         | 12 hrs. 60° C.  |                                  | 23.1                    |
| 4           | 17                                         | 10 min. 125° C. |                                  | 29.9                    |
| 5           |                                            |                 | 6                                | 5.2                     |
| 6 Untreated |                                            |                 |                                  | 24.9                    |

75 The flannel had retained its original desirable

hand and the draping characteristics of the urea-formaldehyde containing fabrics was greatly enhanced.

*Example 3.*—A set of samples was prepared exactly as described in Example 2 except that 15% urea-formaldehyde condensation product was applied to the fabric instead of 17%. The shrinkage results, etc., are given below.

| Sample No.  | Per Cent Urea-formaldehyde Resin on Fabric | Cure            | Per Cent Polybutadiene on Fabric | Per Cent Area Shrinkage |
|-------------|--------------------------------------------|-----------------|----------------------------------|-------------------------|
| 1           | 15                                         | 12 hrs. 60° C.  | 6                                | 6.9                     |
| 2           | 15                                         | 10 min. 125° C. | 6                                | 6.5                     |
| 3           | 15                                         | 12 hrs. 60° C.  | —                                | 28.7                    |
| 4           | 15                                         | 10 min. 125° C. | —                                | 31.5                    |
| 5           | —                                          | —               | 6                                | 8.0                     |
| 6 Untreated | —                                          | —               | —                                | 33.4                    |

*Example 4.*—A set of samples was prepared exactly as described in Example 2 except that 12% urea-formaldehyde condensation product was applied to the fabric instead of 17%.

A firm hand was imparted to the fabric. The samples which were treated with the polybutadiene emulsion showed superior resistance to felting and shrinkage on laundering.

The results of a three-hour wash best are given herewith.

| Sample No.  | Per Cent Urea-formaldehyde Resin on Fabric | Cure            | Per Cent Polybutadiene on Fabric | Per Cent Area Shrinkage |
|-------------|--------------------------------------------|-----------------|----------------------------------|-------------------------|
| 1           | 12                                         | 12 hrs. 60° C.  | 6                                | 5.4                     |
| 2           | 12                                         | 10 min. 125° C. | 6                                | 4.9                     |
| 3           | 12                                         | 12 hrs. 60° C.  | —                                | 27.4                    |
| 4           | 12                                         | 10 min. 125° C. | —                                | 29.1                    |
| 5           | —                                          | —               | 6                                | 6.9                     |
| 6 Untreated | —                                          | —               | —                                | 31.0                    |

*Example 5.*—A treating bath was prepared by dissolving 120 parts dimethylolurea and 30 parts of urea in 850 parts of water. To this solution was added 5% ammonium sulfate, based on the weight of the urea-formaldehyde condensation product and 2% sodium lauryl sulfate based on the total weight of the pad liquor. Wool flannel squares 10" x 10" in size were weighted and immersed in the liquor. After thorough penetration had taken place the excess liquor was removed by passing the fabric through squeeze rollers. The goods were weighed again and from the weight increase as well as the strength of the solution the amount of urea-formaldehyde on the fabric was calculated. After drying, two swatches were cured at 125° C. for ten minutes while the other two were cured for twelve hours at 60° C.

One piece each cured at 60° C. and at 125° C. were treated with the polybutadiene emulsion of Example 1, as follows:

The two pieces of wool weighing 24.2 parts were put into a bath consisting of 485 parts of water at 60°-70° C. and 4.8 parts of 50% acetic acid. After five minutes, 4.8 parts of the polybutadiene emulsion was added, this amount containing a weight of polymer corresponding to 6% of the weight of the samples. Five minutes later 2.4 parts of anhydrous sodium sulfate in the form of a 10% solution were added and these additions were repeated until the bath cleared completely, indicating complete exhaustion. The samples had been agitated continuously throughout the application, and the temperature kept between 65 and 70° C.

The samples were rinsed with warm water and dried.

A piece of wool to which no urea-formaldehyde had been applied was also treated with the polybutadiene emulsion according to the procedure as outlined above.

All samples, as well as an untreated swatch were washed for three hours in a washing machine, containing 35 parts of powdered neutral soap in 18,500 parts of water at 65° C. After rinsing and drying the samples were remeasured. The results have been tabulated below.

| Sample No.  | Per Cent Urea-formaldehyde Resin on Fabric | Cure            | Per Cent Polybutadiene on Fabric | Per Cent Area Shrinkage |
|-------------|--------------------------------------------|-----------------|----------------------------------|-------------------------|
| 1           | 20                                         | 12 hrs. 60° C.  | —                                | 5                       |
| 2           | 20                                         | 10 min. 125° C. | —                                | 5                       |
| 3           | 20                                         | 12 hrs. 60° C.  | —                                | 22.4                    |
| 4           | 20                                         | 10 min. 125° C. | —                                | 26.1                    |
| 5           | —                                          | —               | —                                | 5                       |
| 6 Untreated | —                                          | —               | —                                | 31.6                    |

The urea-formaldehyde treated fabrics had superior draping qualities.

*Example 6.*—A set of samples was prepared exactly as described in the previous example with the exception that only 14% of the urea-formaldehyde condensation product was applied instead of 20%.

The fabrics had good draping qualities and good shrink resistance, as well as superior resistance to felting. The degree of felting, etc. occurring after a three-hour laundering is tabulated below.

| Sample No.  | Percent Urea-formaldehyde Resin on Fabric | Cure            | Percent Polybutadiene on Fabric | Degree of Felting |
|-------------|-------------------------------------------|-----------------|---------------------------------|-------------------|
| 1           | 14                                        | 12 hrs. 60° C.  | —                               | 5                 |
| 2           | 14                                        | 10 min. 125° C. | —                               | 5                 |
| 3           | 14                                        | 12 hrs. 60° C.  | —                               | 5                 |
| 4           | 14                                        | 10 min. 125° C. | —                               | 5                 |
| 5           | —                                         | —               | —                               | 5                 |
| 6 Untreated | —                                         | —               | —                               | 5                 |

*Example 7.*—A similar set of samples was prepared and tested but in this case only 10% urea-formaldehyde condensation product was applied to the fabric. In all other respects the procedure was identical to the one used in Example 5.

Excellent draping effects were imparted to the treated fabrics, as well as good shrink resistance to the samples to which polybutadiene had been applied.

| Sample No.  | Percent Urea-formaldehyde Resin on Fabric | Cure            | Percent Polybutadiene on Fabric | Degree of Felting |
|-------------|-------------------------------------------|-----------------|---------------------------------|-------------------|
| 1           | 10                                        | 12 hrs. 60° C.  | —                               | 5                 |
| 2           | 10                                        | 10 min. 125° C. | —                               | 5                 |
| 3           | 10                                        | 12 hrs. 60° C.  | —                               | 5                 |
| 4           | 10                                        | 10 min. 125° C. | —                               | 5                 |
| 5           | —                                         | —               | —                               | 5                 |
| 6 Untreated | —                                         | —               | —                               | 5                 |

*Example 8.*—Three squares of wool flannel, measuring 10" x 10", were treated with 5% polybutadiene dispersion according to the procedure outlined in Example 5.

After rinsing and drying one sample was immersed in a 10% aqueous alkylated melamine formaldehyde solution. This solution was pre-

pared by diluting the alkylated melamine formaldehyde solution, known commercially as "Resloom M75" which contains 55% solids, in the ratio of 2 parts of "Resloom" to 9 parts of water, and the other one was immersed in a solution of urea-formaldehyde prepared by dissolving equimolecular quantities of dimethylolurea and urea in water to give a solution containing 10% solids. To the "Resloom" solution 3% of diammonium phosphate was added as a catalyst. For the same purpose 5% ammonium sulfate was added to the urea-formaldehyde solution. Both percentages were based on the weight of the solids present in the solutions.

After complete penetration had taken place the excess liquor was removed by passing the samples through squeeze rollers. After drying the swatches were cured at 125° C. for ten minutes. From the amount of liquid pick-up as well as from the concentration of the solution, the amount of resin deposited on the fabric was determined.

Two additional pieces of flannel were treated in the same manner with "Resloom" and urea-formaldehyde solutions without having had the polybutadiene treatment first.

All pieces as well as an untreated piece were washed for three hours in a mechanical washing machine. After drying they were remeasured and the area shrinkage was calculated.

A résumé of the various treatments as well as the area shrinkage is given herewith.

The area shrinkage was as follows:

| Sample No. | Treated with                             | Area Shrinkage |
|------------|------------------------------------------|----------------|
| 1          | 6% polybutadiene + 10% "Resloom"         | 0.7            |
| 2          | 6% polybutadiene + 10% urea-formaldehyde | 1.5            |
| 3          | 6% polybutadiene                         | 6.4            |
| 4          | 10% "Resloom"                            | 11.2           |
| 5          | 10% urea-formaldehyde                    | 30.5           |
| 6          | Control                                  | 31.1           |

Example 10.—Samples of wool flannel were treated with aqueous alkylated melamine formaldehyde solutions, prepared from a commercial product known to the trade as "Resloom M75." This product contained 55% solids and was diluted with water so as to form solutions which contained 19, 14, 10 and 5% solids and to which 3% of diammonium phosphate, based on the weight of the solids, had been added. The excess solution was removed by passing through squeeze rollers, the fabric retaining 100% of its weight of solution. After drying, all samples were cured for ten minutes at 125° C.

A similar set of samples was prepared and after curing, these swatches were immersed in a solution which had been obtained by diluting an aqueous polybutadiene dispersion with water to such an extent, that the resulting solution contained 6% of the polymer. The samples

| Sample No.  | Per cent Polybutadiene On Fabric | Cure            | Per Cent Resin Treatment On Fabric | Per Cent Area Shrinkage |
|-------------|----------------------------------|-----------------|------------------------------------|-------------------------|
| 1           | 5                                | 10 min. 125° C. | 9% "Resloom"                       | 0.9                     |
| 2           | 5                                | 10 min. 125° C. | 10.8% urea-formaldehyde            | 0.5                     |
| 3           | 5                                | 10 min. 125° C. | 10.8% "Resloom"                    | 2.3                     |
| 4           | 5                                | 10 min. 125° C. | 11.0% urea-formaldehyde            | 20.6                    |
| 5           | 5                                | 10 min. 125° C. |                                    | 23.3                    |
| 6 Untreated |                                  | 10 min. 125° C. |                                    | 24.6                    |

Example 9.—Five solutions were made up as follows:

| Solution No.                                                   | 1        | 2        | 3        | 4     | 5     |
|----------------------------------------------------------------|----------|----------|----------|-------|-------|
| Polybutadiene (25% dispersion)                                 | Parts 24 | Parts 24 | Parts 24 | Parts |       |
| Alkylated Melamine formaldehyde ("Resloom M75" 55% solids)     | 18.2     | -----    | -----    | 18.2  | ----- |
| Urea formaldehyde condensation product <sup>1</sup> 15% solids | 66.7     | -----    | -----    | 66.7  | ----- |
| Diammonium phosphate                                           | .3       | -----    | .3       | .5    | ----- |
| Ammonium sulfate                                               | .5       | -----    | -----    | .5    | ----- |
| Water                                                          | 67.5     | 88       | 76       | 81.5  | 32.8  |

<sup>1</sup> The urea formaldehyde condensation product solution was prepared by dissolving equimolecular quantities of dimethylol urea and urea in sufficient water to yield a solution containing a total of 15% solids.

Measured swatches of wool were thoroughly wet out, the excess liquor removed by passing the fabric through squeeze rollers, and the amount of liquid pick-up determined. From the pick-up, the amount of polymer and/or resin deposited on the wool was calculated. These amounts as well as the shrinkage may be found in the table below. The pieces were dried, and those containing the urea-formaldehyde and the alkylated melamine formaldehyde condensation products were cured for ten minutes at 125° C. After curing, these pieces had a normal, full hand and pleasing draping characteristics.

All pieces, including an untreated piece, were washed for three hours and remeasured.

were permitted to remain in contact with the bath until they were completely wetted out. The excess liquid was then removed by passing the swatches through squeeze rollers.

The samples were found to have doubled in weight, and since the pad liquor contained 6% of polymer, 6% polybutadiene was deposited on the fabric.

All samples were measured before and after laundering and the percent area shrinkage was determined. The results were as follows:

| Sample No. | Treated with                                           | Area Shrinkage |
|------------|--------------------------------------------------------|----------------|
| 1          | 10% alkylated melamine formaldehyde                    | 10.5           |
| 1a         | 19% alkylated melamine formaldehyde + 6% polybutadiene | 4.5            |
| 2          | 14% alkylated melamine formaldehyde                    | 17.9           |
| 2a         | 14% alkylated melamine formaldehyde + 6% polybutadiene | 4.2            |
| 3          | 10% alkylated melamine formaldehyde                    | 21.0           |
| 3a         | 10% alkylated melamine formaldehyde + 6% polybutadiene | 4.2            |
| 4          | 5% alkylated melamine formaldehyde                     | 23.3           |
| 4a         | 5% alkylated melamine formaldehyde + 6% polybutadiene  | 6.7            |
| 5          | Untreated                                              | 30.1           |

Example 11.—A solution of a melamine-formaldehyde condensation product was prepared by dissolving with heat melamine and formaldehyde in a molar ratio of 1 to 3 in sufficient water to

## 15

give a product containing 10% solids. On cooling 5% of ammonium sulfate based on the weight of the solids was added as a catalyst.

Two swatches of wool 10" x 10" were weighed and immersed in this solution. After the samples had wetted out thoroughly, the excess solution was removed by passing them through squeeze rollers. The samples were reweighed, dried and cured by allowing them to remain at room temperature for 24 hours.

The solution was then diluted with water so as to contain 5% melamine-formaldehyde condensation product and an additional two samples were heated according to the procedure as outlined above.

In each case the fabric increased 100% in weight.

After the curing one sample each containing 10% and 5% of melamine formaldehyde as well as an untreated swatch were treated with the 6% polybutadiene emulsion of Example 1.

The emulsion was applied by padding and in this manner 6% polybutadiene was deposited on the fabric. The samples, which included those which were treated with melamine-formaldehyde only, as well as a measured untreated swatch, were then dried and laundered for three hours. After drying, the swatches were remeasured and the amount of area shrinkage was calculated in per cent.

A résumé of the treatment and the shrinkage control follows:

| Sample No.  | Per Cent Melamine-formaldehyde Resin on Fabric | Per Cent Polybutadiene on Fabric | Per Cent Area Shrinkage |
|-------------|------------------------------------------------|----------------------------------|-------------------------|
| 1           | 10                                             | 6                                | 10.3                    |
| 2           | 10                                             | 6                                | 7.2                     |
| 3           | 5                                              | 6                                | 23.9                    |
| 4           | 5                                              | 6                                | 5.6                     |
| 5           | 5                                              | 6                                | 4.4                     |
| 6 Untreated |                                                |                                  | 25.5                    |

## 16

shrink resistance were imparted to the fabric as tabulated below.

| Sample No.  | Per Cent Urea-formaldehyde Resin on Fabric | Per Cent Polybutadiene on Fabric | Per Cent Area Shrinkage |
|-------------|--------------------------------------------|----------------------------------|-------------------------|
| 1           | 10                                         | 6                                | 23.3                    |
| 2           | 10                                         | 6                                | 0.8                     |
| 3           | 5                                          | 6                                | 22.3                    |
| 4           | 5                                          | 6                                | 5.7                     |
| 5           | 5                                          | 6                                | 6.2                     |
| 6 Untreated |                                            |                                  | 24.4                    |

## 15

*Example 13.*—A solution of a melamine-formaldehyde condensation product was prepared by dissolving with heat melamine and formaldehyde in a molar ratio of 1 to 4 in sufficient water to give a product containing 10% solids. After the solution cooled, ammonium sulfate was added to the solution to the extent of 5% based on the weight of the solids. Two weighed and measured swatches of wool flannel were padded with these solutions, the excess being removed through squeeze rollers, dried and cured for 24 hours at room temperature.

One of these wool squares was then padded from a 6% polybutadiene emulsion and permitted to dry. Another two swatches were treated with a 10% solution of a melamineformaldehyde condensation product prepared by dissolving melamine and formaldehyde condensation product prepared by dissolving melamine and formaldehyde in a molar ratio of 1 to 3. No catalyst was added to this solution. The treated wool pieces were cured for 24 hours at room temperature. One of these pieces was also treated with 6% polybutadiene and dried. Finally all these swatches, as well as a swatch of wool treated with 6% polybutadiene and an untreated square were washed and measured for shrinkage control. A good full hand was imparted to the fabric which had excellent draping qualities.

| Sample No.  | Per cent Melamine-Formaldehyde Resin on Fabric | Ratio Melamine to Formaldehyde | Catalyst            | Per cent Polybutadiene on Fabric | Per cent Area Shrinkage |
|-------------|------------------------------------------------|--------------------------------|---------------------|----------------------------------|-------------------------|
| 1           | 10                                             | 1 to 4                         | 5% ammonium sulfate | 6                                | 26.0                    |
| 2           | 10                                             | 1 to 4                         | do                  | 6                                | 1.7                     |
| 3           | 10                                             | 1 to 3                         | None                | 6                                | 26.7                    |
| 4           | 10                                             | 1 to 3                         | do                  | 6                                | 1.7                     |
| 5           |                                                |                                |                     | 6                                | 3.2                     |
| 6 Untreated |                                                |                                |                     |                                  | 28.5                    |

The samples which were treated with the melamine-formaldehyde resin had a desirable drape and a full hand.

*Example 12.*—A similar set of samples was prepared and tested, but in this case the solution of urea-formaldehyde condensation product of Example 1 was substituted for the melamine-formaldehyde of the previous example. In all other respects the procedure was identical to the one used in Example 11. Superior draping characteristics, and in some instances good felting and

Having thus set forth my invention, I claim:

1. A bath for shrinkproofing wool while retaining substantially normal hand which comprises an aqueous substantially stable emulsion containing a synthetic butadiene-1,3 polymer of 100% polymerization and at least one of the urea-formaldehyde and melamine-formaldehyde resins, the ratio of resin to polymer being from 4:1 to 1:1.2 for the urea-formaldehyde resin and from 3:1:1 to 1:1.2 for the melamine-formaldehyde resin, the polymer and resin being present

in amount to give 1 to 50% by weight of polymer and resin deposition on the wool, the amount of polymer being from 2 to 15% by weight on the wool, the bath also containing a non-cationic emulsifying agent and at least 25% by weight on the polymer of a water-soluble neutral salt of an alkali metal as conditioning electrolyte and having a pH below about 7.

2. A bath as set forth in claim 1, in which the emulsifying agent is anionic.

3. A bath as set forth in claim 1, which includes a curing catalyst for the resin.

4. A bath as set forth in claim 1, in which the resin is a urea-formaldehyde resin and the resin to polymer ratio is from 4:1 to 1:1.2.

5. A bath as set forth in claim 1, in which the resin is a melamine-formaldehyde resin and the resin to polymer ratio is from 3:1:1 to 1:1.2.

JOHN B. RUST.

#### REFERENCES CITED

The following references are of record in the file of this patent:

#### UNITED STATES PATENTS

| Number    | Name           | Date           |
|-----------|----------------|----------------|
| 2,173,242 | Young          | Sept. 19, 1939 |
| 2,211,959 | Maney          | Aug. 20, 1940  |
| 2,299,786 | Battye et al.  | Oct. 27, 1942  |
| 2,340,358 | Young          | Feb. 1, 1944   |
| 2,384,880 | Britton et al. | Sept. 18, 1945 |
| 2,405,038 | Jennings       | July 30, 1946  |

#### OTHER REFERENCES

15 Rubber Age (N. Y.) vol. 48 of 1940, pp. 23-25.